# EUROPEAN PATENT SPECIFICATION

(11) **EP 0 127 620 B1**
(45) Date of publication and mention of the grant of the patent: **23.09.1987**
(21) Application number: 83900525.3
(22) Date of filing: 01.12.1982
(51) Int. Cl.: C25D 5/48, C25D 7/00, C25D 15/00

(54) **ELECTROLYTIC CODEPOSITION OF ZINC AND GRAPHITE AND RESULTING PRODUCT**
ELEKTROLYTISCHER ZUSAMMENNIEDERSCHLAG VON ZINK UND GRAPHIT UND SO ERHALTENER GEGENSTAND
COSEDIMENTATION ELECTROLYTIQUE DE ZINC ET DE GRAPHITE, AINSI QUE LE PRODUIT RESULTANT

(43) Date of publication of application: 12.12.1984
(73) Proprietor: FORD MOTOR COMPANY, Dearborn, MI 48121 (US); FORD MOTOR COMPANY LIMITED, Brentwood, Essex CM13 3BW (GB); FORD-WERKE AKTIENGESELLSCHAFT, 50725 Köln (DE); FORD FRANCE SOCIETE ANONYME, 92506 Rueil Malmaison Cedex (FR)
(72) Inventor: DONAKOWSKI, William, A., Dearborn Heigths, MI 48127 (US); MORGAN, John, R., Southfield, MI 48034 (US)
(74) Representative: Messulam, Alec Moses
(86) International application number: US8201689
(87) International publication number: WO8402149

## Description

Automotive metal fasteners are usually coated or plated to enhance various characteristics such as resistance to corrosion, resistance to seizing/galling, low fastening friction, economy, solderability, and resistance to the stick-slip phenomenon (which is a repeated sticking followed by repeated slipping during fastener tightening operations).

To provide resistance to corrosion, it has become conventional in the automotive fastener art to coat the fastener with phosphate and oil or to electroplate with zinc. Unfortunately such coated or plated fasteners are subject to the stick-slip phenomenon when the fastener is tightened with power tools, causing the desired torque loading to sometimes be off target. This stick-slip phenomenon is in part related to a relatively high coefficient of friction for the coating or plating. As the power tool turns the coated or plated nut onto a threaded bolt, the phosphate or zinc is spalled off and collects in small masses to form miniature wedges between the threads. The torque tool will shut off prematurely in response to the effect of these wedges, leaving the mechanical assembly improperly secured under such circumstances, which assembly must 1₃ter be reworked when identified by an inspecting system.

To obviate the stick-slip problem and to impart a lower coefficient of friction to the coating or plating, cadmium has been employed to impart lubricity and good sacrificial corrosion protection, particularly in a marine environment (see Modern Electroplating, by F. A. Lowenheim, published by John Wiley & Sons, 3rd Edition, p. 663, 1974). However, cadmium is subject to two disadvantages: (a) it has a toxic effect during processing, and (b) it is significantly expensive.

A codeposited material which would combine the low coefficient of friction of each of its constituent ingredients would appear to offer potential in meeting the various characteristics desired for an automotive fastener; but this has not necessarily proven to be the case. Experimentation with codeposits of metal and inorganic particles has been reported in the literature.

In an article entitled "Codeposition of Finely Dispersed Inorganic Particles" by Tomaszewski et al, published in Plating, Vol. 56, p. 1234. November 1969, the author investigated using acidic copper plating and acid nickel baths containing various inorganic particles including graphite, MoS₂, BaS0₄, SrS0₄, AI₂0₃, _{Ti02}, _{Zr02}, H2AI2Si20a' _{H20}, _{PbS04}, _{Pb3}(P0₄)₂, Ce0₂, BN, B₆C, B, Si, and Si0₂.

Some of these codeposited particles can be considered nonconductive and normally would not respond to the normal electrolytic action, but it was found that even graphite would plate or codeposit under very strained and undesirable conditions with nickel. The metal matrix and codeposited particles were viewed as to their antifriction, antiseizing, and dry lubrication properties and found them not lower than zinc or cadmium. No investigation was made of the mode of corrosion of such codeposits. Without exploring proper processing parameters, the author concluded that codeposition was feasible only at conventional metal plating parameters. Similar observations were made by Parker as to electroless nickel deposits, entitled "Hardness and Wear Resistance Tests of Electroless Nickel Deposits", Journal of Plating, Vol. 61, p. 834, September 1974. None of the codeposits investigated by these scientists provided a low enough coefficient of friction which would be comparable to cadmium plating now used in the art. Thus these coatings were lacking in a good antigalling characteristic and good corrosion resistance. Nickel does not fail by a sacrifical corrosion mode and thus requires inordinately thick deposits to act as a physical barrier and protect the substrate. The low coefficient of friction of each of the constituent ingredients did not necessarily add up to a total lower coefficient of friction for the codeposited material. In addition, each codeposit lacked good cathode efficiency and low material cost.

One group of investigators, Messrs. Chouse and Ramachandren, explored the "Antifriction Properties of Electrodeposited Composites of Graphite or Molybdenum Disulfide with Copper", Journal of Metal Finishing, Vol. 78, p. 85, June 1981. The amount of second phase material (graphite or MoS₂) was found to have a slight effect on total coefficient of friction of the combined material but insufficient to make the codeposit have an improved coefficient of friction comparable to cadmium.

Chemical Abstract volume 87, 1977 Page 218 Abstract 42822w discloses surface treatment of steel plate suitable for press forming wherein steel plates are coated first with Zn by galvanisation and then with Zn-graphite by treating the plates in plating solution.

DE-A-2325559 discloses a coating of Zn and graphite. Zn and graphite are simultaneously electrodeposited.

What is needed by the prior art is a codeposited material and accompanying method of depositing such material, which material is equal to or better than cadmium plating with respect to the coefficient of friction, has no toxic effects, is superior in antiseizing and antigalling characteristics, is high in cathode efficiency, offers reasonably good corrosion resistance in a nonmarine environment, and is solderable.

According to the invention there is provided a method of electrodepositing zinc and graphite onto conductive metal substrate by the use of an electrolytic cell having a zinc anode and the metal substrate connected as a cathode, the method comprising the steps of immersing said substrate in a cleansed condition into an acid/zinc plating electrolyte containing at least 40 g/I zinc ions and 30-110 g/I insoluble bulk graphite, said electrolyte having a pH of 5-5.7 and energizing said electrolytic cell at a sufficient current density to plate out zinc onto said surface without burning while continuously agitating said graphite into uniform suspension throughout said electrolyte, said agitation being periodically interrupted to allow said graphite to settle and comingle with said zinc as it is plating out on said cathode, the codeposit of zinc and graphite on said substrate containing uniformly distributed graphite in an amount of 30-48% by weight of the codeposit, a coefficient of friction equal to or less than .130, at a plated thickness of 0.00127 cms (0.0005"), showing no red rust'in a salt spray environment for at least 72 hours and no destruction due to corrosion in an industrial environment containing sulphur dioxide after four months.

To enhance the corrosion resistance of the codeposited material, the codeposit may be subject to an additional step of dipping into a chromate passivation solution for a period of 10-30 seconds in order to form a conversion zinc chromate coating on the outer layer of said codeposit. Preferably the layer of zinc chromate has a thickness of .00005 cms (.00002") so that optimally the coated combination will exhibit consistent torque performance at a torque load of 40 pounds, a coefficient of friction of about .112 or less, and no red rust in a salt spray environment for at least 120 hours. When the codeposited coating is applied to a threaded fastener, the fastener will preferably exhibit a consistent torque tension relationship during tightening and have good solderability characteristics using either a resin solder cord or a zinc chloride containing flux.

Preferably the conductive metal substrate is a metallic threaded fastener which may be comprised of steel, copper, nickel, brass, bronze, zinc and aluminum. The agitation is preferably interrupted for 15-60 seconds at intervals of 15-80 seconds. It is advantageous if the particle size of the graphite employed is of an extremely fine character, and preferably is of a colloidal nature having a particle size of 1-25 microns.

Preferably the electrolyte is of the acid chloride type, created by either mixing 70-85 g/I zinc chloride with 100150gII of potassium chloride, or 45-110 g/l of zinc chloride when dissolved with 100-200 g/I of sodium chloride. The acid chloride bath contains also boric acid in an amount of 26―40 g/I. Optimally the electrolyte may be improved by incorporating a grain refiner in the form of gelatin in an amount of .41 g/I of electrolyte, and a cationic surfactant in the form of cocamine acetate in an amount of .1-.4 g/I of electrolyte.

Advantageously the cleaning of the substrate may include immersion in a caustic cleansing solution to remove oils and other organic materials followed by a clean water rinse, and then immersion in a pickling solution to remove any oxides thereon, again followed by water rinse. In the plating of a batch of threaded metal fasteners, it is desirable to employ a barrel plating process whereby the apparatus is comprised of a mechanically rotated barrel which is perforated and contains a metallic plate bolted to the bottom of the barrel which in turn is connected to a commutator ring on the outside of the barrel. The barrels are made of inert material such as polypropylene. The cathode contact with the fasteners is usually made by metal discs on the bottom of the cylinder. The electrolyte permeates the barrel through the perforations and the anode is suspended just below the level of the solution.

The invention will now be described further by way of example with reference to the accompanying drawings in which:
Figure 1 is a schematic illustration of a barrel plating apparatus and tank set-up used to carry out a process mode in conformity with this invention;
Figures 2 and 3 are enlarged schematic illustrations of a portion of a coating showing inorganic particles embedded in the coating, Figure 2 employing conductive particles and Figure 3 using nonconductive inorganic particles;
Figure 4 is a graphical illustration showing the variation of coefficient of friction as a function of the type of material employed in the coating, particularly the concentration of graphite in a codeposit of zinc and graphite;
Figure 5 is a graphical illustration of the deposition rate or volume of the codeposited materials of this invention as a function of the current density;
Figures 6-8 each respectively illustrate a graphical illustration of torque and tension as a function of the angle of rotation of a fastener coated respectively with phosphate and oil (Figure 6), zinc and graphite, codeposit with a chromate outer coating (Figure 7), and a cadmium plate with a chromate outer coating (Figure 8);
Figures 9-11 each respectively illustrate a scanning electron microscope photograph (at 100x) of coatings prepared in accordance with the process teaching of this invention, Figure 9 illustrating a coating prepared with a concentration of 120 g/I of graphite in the electrolyte, Figure 10 illustrating a coating prepared from a 75 g/I concentration of graphite in the electrolyte, and Figure 11 illustrating a concentration of 50 g/I graphite in the electrolyte; and
Figure 12 is an electron scanning microscope photograph of a section of a coating prepared in accordance with this invention showing the various layers of the coating as labeled.

This invention has discovered that a codeposit of zinc and graphite with a critically high content of graphite will provide an unusually good combination of physical characteristics, including an ultralow coefficient of friction. The physical characteristics may comprise anticorrosion properties, good solderability, economy of processing and little or no stick slip problem. The codeposit of zinc and graphite has particular utility in the coating of fasteners, pins and gears.

A preferred method mode for obtaining the codeposit of this invention is as follows.

### Apparatus preparation

Prior to performing the steps of-the method, a processing and electrolytic plating system is prepared. As shown in Figure 1, a barrel plating mode may be employed whereby rotatable cylinders 10, constructed of acid resistant, nonabsorbant material (such as polypropylene, resin bonded fiberglass, hard rubber, PVC, lucite, and phenolic laminates) are used to contain the parts to be plated while being tumbled. The cylinders are perforated and are mounted for rotation upon a horizontal axis, the trunions 11 for the axis being supported in a carriage 12 which is moved from tank to tank and is lowered into each tank for treatment therein. The series of tanks that may be employed with this method, and barrel plating apparatus, include a series of cleaning and rinsing tanks (not shown, which are interposed between process tanks). One or more of electrolytic plating tanks 13-14-15 are employed, followed by a suitable rinse tank 16. Only the electrolytic plating tanks are energized and contain an electrolyte. The parts, such as metal fasteners, are loaded in a bulk fashion into the cylinder through an access door thereof; the parts are connected as a cathode in the electrolytic plating cell by use of a metal plate bolted to the bottom of the barrel for contact with the batch of parts. The plate is connected by slip ring to an outside electrical supply. The anode can comprise a plurality of zinc elements extending into the bath containing the electrolyte solution and into which the barrels are lowered.

Proceeding now with the method steps of this invention:

### 1. Cleaning the metal to be plated

The substrate, or, in this case, a bulk quantity of metallic fasteners, is loaded into the barrel plating cylinder and carried through a series of cleaning tanks, which may preferably comprise a first bath having a highly alkaline solution effective to remove oil and gum deposits on the metallic substrate. The alkaline cleansed metal substrate is then rinsed by use of conventional tap water and then immersed in a pickling solution containing a concentration of about 30% hydrochloric acid, which is effective to remove oxides, followed by a conventional water rinse.

### 2. Immersing the substrate in suitable plating electrolyte

Prior to immersing the cleansed substrate into an acid zinc plating electrolyte for depositing a codeposit, the parts may preferably be preplated with .0005 cms (0.0002") zinc in a conventional acid zinc plating electrolyte.

The electrolyte for the codeposit contains 40 g/I zinc ions and 30-110 g/l insoluble bulk graphite. The zinc ions are obtained in the electrolyte by introducing a zinc anode into the bath solution; the bulk graphite is preferably introduced in a fine grade condition, optimally colloidal graphite, having a particle size in the range of 1-25 microns. Crude foundry grade graphite is operable within the scope of this invention, crude graphite having an average particle size of 25-100 microns. Utilizing the finer colloidal graphite will obtain a much smoother codeposit having typically an average particle size of 2 microns. If the graphite is added to the electrolyte in amounts less than 30 g/l, a noticeable increase in the coefficient of friction of the codeposit will result and make the coating less effective in performing as a low friction composite. If the graphite is added to the solution and maintained in a suspension quantity of greater than 110 g/I, the graphite will plate out in an amount which will be greater than 50% of the codeposit and thus substantially reduce the ability of the codeposit to have anticorrosion characteristics attributable to the presence of zinc.

Preferably the acid zinc electrolyte is prepared by adding to an aqueous solution 45-110 g/I zinc chloride and 100-200 g/I sodium chloride. The pH of such acid bath should be maintained in the range of 5-5.7 and optimally about 5.3. This bath has the advantage of plating on difficult metals and will have an almost 100% cathode efficiency. Alternatively, the acid chloride bath may be prepared by using 70-85 g/I zinc chloride and 100-150 g/I of potassium chloride. Boric acid in the range of 26-40 g/I may be added as a buffering agent.

To improve the grain refinement of the resulting codeposit, .4-1 g/I of unflavored gelatin may be added to the electrolyte. Additionally, .1-4.0 g/I cocamine acetate (having the molecular formula of C₁₂H₂,NH₃) is added, which serves to facilitate the deposition of nonconductive particles.

The pH range should be regulated as given. If higher than such range, zinc hydroxide will form which is undesirably insoluble. If lower than 5, the acidity of the electrolyte will affect cohesion. The electrolyte should be maintained in a temperature range of 24-32°C (7590°F).

It is essential to employ an acid zinc plating electrolyte so as to enable the cohesion of the inert graphite particles to facilitate forming the codeposit.

### 3. Energizing the electrolytic cell

The electrolytic cell is energized at a sufficient current density to plate the zinc onto the substrate without burning while continuously agitating the graphite into suspension throughout said electrolyte. The agitation is periodically interrupted to allow the graphite to settle and comingle with the zinc as the plating takes place on the cathode. Preferably the agitation is carried out by the use of air pulsing and is interrupted for periods of 15―60 seconds at intervals of 15-180 seconds. During all other times the air pulsing is on. The current density is preferably employed in the low range of 1-20 amps per square foot (.1-2.0 amps/dm²). If the current density is lower than this value, insufficient plating zinc will take place. If the amperage is much higher, there is a tendency for the zinc to be burned during its electroplating process. The generally inert graphite particles will accept an electrostatic charge that is promoted by the electrolytic cell. The charge is very light and therefore migration of the particles to the cathode is extremely sensitive. It is important that agitation be employed so that there is, in suspension, the critical range of 30-110 g/l of graphite. The amount of agitation to maintain such suspension is determined by the specific gravity of the electrolyte.

As shown by the comparison of Figures 2 and 3, the surface profile of a codeposited material will have a surface roughness which will vary depending upon whether highly conductive particles are entrapped by the metal or whether the particles are substantially nonconductive. In Figure 2, cobalt particles are enveloped by the primary plating metal causing a relatively rough surface to be formed. Graphite particles, which carry a low level of electrostatic charge, are embedded within the plating metal primarily by a settling action and are not enveloped by the plating metal resulting in a much smoother finish (see Figure 3).

The rate of zinc metal deposition affects the entrapment rate of the graphite particles during the coating of the cathode. There is a relatively low level of electrostatic attraction between the graphite particles and the cathode, and this electrostatic force can be easily interrupted or overcome by a mechanical agitation force. It has been found that by controlling the current density (which controls the deposition rate of the metal indirectly), and controlling the force of agitation which disrupts such deposition, the graphite deposition rate and graphite particle volume can be optimized (see Figure 5). If a current density of between .8―1.6 amps/dm² is employed, the best graphite rate as well as graphite volume deposition is obtained. This is conditioned upon the interruption of the agitation force for 15-60 second periods at intervals of 15-180 seconds to allow for such deposition rate to take place.

### 4. Chromate outer coating

It is desirable to dip the electroplated codeposit in a solution containing an acid chromate for a period of 10―45 seconds to form a very thin chromate outer coating on the metal substrate. The chromate should typically have a thickness of 2.54x2-⁵cms (2-^{S}inches) thick. The zinc/graphite plated part is dipped in a chromating solution consisting of 30 g/f chromic acid, 10 cc/I phosphoric acid, 5 cc/I hydrochloric acid, 5 cc/I nitric acid, and 5 cc/I sulfuric acid for a period of about 30 seconds, followed by a warm rinse of about 30 seconds. When the solution has a pH range of 1.02.0, an olive drab chromate coating will be obtained which has the characteristic of good corrosion protection. The color of such chromate conversion coating is dependent upon the thickness of the coating and also the trivalent chromium content of the bath (0.1-4 g/I). The color is relatively clear and bright for the thinnest coating, proceeding to a blue-bright, then yellow iridescent in progressively thicker coatings, to the heaviest coating of brown or olive drab colors. A more complete disclosure of the application of chromate coatings is set forth in "Conversion Coatings-Chromate Films", by L. F. Spencer, Metal Finishing, pp. 58-65, January 1960 (which disclosure is incorporated herein by reference).

The chromate conversion coating on the codeposit of this invention renders exceptionally good corrosion resistance because of (a) the corrosion inhibiting effect of hexavalent chromium contained in the chromate film, and (b) to the physical barrier presented by the chromate film itself. The film is formed by the chemical reaction of the hexavalent chromium with the zinc metal surface in the presence of activators in the acid solution. The hexavalent chromium is partially reduced to trivalent chromium during the reaction with a concurrent rise in pH, forming a complex mixture consisting largely of hydrated basic chromium chromate and hydrous oxides of both chromium and the zinc metal. It is important that the pH of the treatment solution be maintained in the critical range of 1.0-2.0 to obtain an appropriate chromate conversion coating. The activators useful in forming the conversion coating include acetate formate, sulphate, chloride, fluoride, nitrate phosphate, and sulphamate ions. For purposes of this invention, the immersion time for a conversion coating herein is relatively short, a period of 20-30 seconds.

### Test samples

A series of samples were prepared in conformity with the preferred mode. Each of the samples were iron based nuts; some preplated with 5 microns zinc, and all plated with 8 microns of zinc/graphite. The zinc/graphite plating solution contained 75 g/I of graphite. The zinc/graphite codeposit in some samples was passivated with a chromate film of a thickness of 0.00005 cms (0.00002"). The samples were subjected to a chemical content analysis to determine the content of graphite and the corresponding coefficient of friction at a torque load of 40 ft/lbs. The solution was varied with a variety of graphite contents; the results of such analysis are shown in the following Table 1.

From such Table it is quite evident that the coefficient of friction of the codeposit of zinc and graphite provides an unusually low coefficient of friction. However, when the graphite content in solution is less than 30 g/l, insufficient graphite is deposited to reduce the coefficient of friction (acceptable is .130r. When the graphite in solution is in excess of 110 g/I, the coefficient of friction again rises inordinately. From this it has been determined that the effective operable range for the graphite in the electrolyte should be 30-110 g/I and preferably 50-75 g/I (see Figure 4). It is significant that the coefficient of friction utilizing this preferred process results in a codeposit that has a coefficient of friction substantially less than alternative coating systems used by the prior art (see the following Table 2).

Some of these samples were also analyzed as to the graphite content in the resultirig coated system as a function of the graphite concentration in the bath solution. The results are shown in Table 3 below.

Each of the samples were analyzed for their ability to resist the stick-slipping problem. Each of the fasteners was subjected to a torqueing test whereby a torque measured in foot/pounds is applied to the fastener and the resulting tension of the fastener is plotted against the degree of angle rotation. As the coated nut is fastened to a connecting rod, loading requirements can vary with severe, jerky vacillations. For a prior art coating system, of phosphate and oil, Figure 6 shows the severe vacillations that are encountered as a result of the stick-slip problem. When the nut is coated with a cadmium deposit the aberrations are removed and there is a smooth torqueing curve without the errative behavior, as shown in Figure 8. This same type of smooth torqueing behavior has been experienced with the zinc/graphite codeposit containing a chromate outer coating; this is shown in Figure 7.

To determine the corrosion resistance of the codeposit of this invention, the samples were subjected to a salt spray test according to the ASTM B117 test procedure in a 5% salt spray test. Nuts plated with 13 microns of zinc/graphite from either 50 or 75 graphite bath solution and passivated with a chromate film, passed 120 hours of the salt spray test (see the following Table 4). Another corrosion test includes the exposure of fasteners mounted on vehicles traveling in the Detroit, Michigan and Buffalo, New York areas of the United States. After one winter of exposure (four months) there was no corrosion on samples plated with zinc/graphite in thicknesses of 0.2-0.7 mil or fasteners plated with 0.5 mil cadmium. These results were obtained on passivated and unpassivated zinc/graphite composites.

These same samples were then subjected to a solderability test. The nuts with various coating systems were tested to investigate their suitability for soldering. As a qualitative evaluation, all of the nuts or screws coated with a zinc+zinc/graphite or zinc/graphite and chromate conversion coating, the solderability was excellent in all cases. However, coating systems of phosphate and oil did not provide good solderability with a resin solder cord nor with a zinc chloride containing flux. Plain steel demonstrated poor solderability with resin solder cord. Thus it has been demonstrated that the codeposit of this invention provides excellent solderability characteristics if that is necessary in the application.

In addition, the codeposit of this invention is dry to the touch, which is often commercially difficult to consistently achieve with fasteners coated with phosphate and oil. The shelf life of the codeposit is excellent, having a life of well over one year, and is economical to finish while presenting no hazards with respect to toxic processing considerations. The raw materials for the system are relatively plentiful.

## Claims

1. A method of electrodepositing zinc and graphite onto conductive metal substrate by the use of an electrolytic cell having a zinc anode and the metal substrate connected as a cathode, the method comprising the steps of immersing said substrate in a cleansed condition into an acid/zinc plating electrolyte containing at least 40 g/1 zinc ions and 30-110 g/I insoluble bulk graphite, said electrolyte having a pH of 5-5.7 and energizing said electrolytic cell at a sufficient current density to plate out zinc onto said surface without burning while continuously agitating said graphite into uniform suspension throughout said electrolyte, said agitation being periodically interrupted to allow said graphite to settle and comingle with said zinc as it is plating out on said cathode, the codeposit of zinc and graphite on said substrate containing uniformly distributed graphite in an amount of 30-48% by weight of the codeposit, a coefficient of friction equal to or less than .130, at a plated thickness of 0.00127 cms (0.0005"), showing no red rust in a salt spray environment for at least 72 hours and no destruction due to corrosion in an industrial environment containing sulphur dioxide after four months.

2. A method as claimed in Claim 1, in which said agitation is periodically interrupted for 15 to 60 second periods at intervals of 15 to 180 seconds.

3. A method as claimed in Claim 1 or 2, in which said bulk graphite has an average particle size of 1-25 microns.

4. Amethod as claimed in any one of Claims 1 to 3, in which said electrolyte is of the acid chloride type constituted by either adding 70-85 g/I zinc chloride with 100-150 g/I potassium chloride, or 45-110 g/l zinc chloride with 100-200 g/I sodium chloride, said electrolyte also containing 26―40 g/I boric acid.

5. A method as claimed in Claim 4, in which said electrolyte additionally contains .4-1 g/I gelatin.

6. A method as claimed in Claim 4, in which said electrolyte additionally contains .1-4.0 g/I cocamine acetate.

7. A method as claimed in any one of the preceding claims in which said electrolytic cell is energized by a current density of 1-20 amps per square foot (.1-2.0 amps/dm²).

8. A method as claimed in any one of the preceding claims in which said agitation is carried out by the use of air pulses into said electrolyte.

9. A method as claimed in any one of the preceding claims, in which said electrolyte is maintained at a temperature of 24-32°C (7590°F).

10. A method as claimed in any one of the preceding claims, in which said metal substrate is selected from the group consisting of steel, copper, nickel, brass, bronze, zinc, and aluminum, as well as conductive plastics.

11. A method as claimed in any one of the preceding claims, in which said process additionally comprises the step of dipping said codeposited material into a chromate solution for a period of 10-30 seconds to form a conversion coating on said codeposit consisting of zinc chromate.

12. A method as claimed in any one of the preceding claims, in which said substrate is a threaded metal fastener.

13. A method as claimed in Claim 12 of electroplating a batch of threaded metal fasteners by the use of a barrel plating apparatus having a perforated barrel within which is introduced the plating electrolyte with the fasteners contacted to constitute a cathode, the method comprising, dipping said barrel contained fasteners sequentially through a series of tanks, the tanks including a caustic cleaning solution, water rinse, a pickling solution for removing oxides, a water rinse, the zinc/graphite plating electrolyte and a water rinse, energizing said zinc/graphite plating electrolyte when said barrel contained fasteners are immersed in said solution, said energization being carried out at a level to plate out zinc on said fasteners without burning, said plating being carried out with the injection of jet streams of compressed air to maintain the graphite continuously in suspension within said electrolyte and interrupting said barrel rotation and air agitation periodically to allow said graphite to migrate and plate out with said zinc on the cathode.

## Patentansprüche

1. Verfahren zur galvanischen Abscheidung von Zink und Graphit auf ein Leitfähiges Metallsubstrat mittels einer Elektrolysezelle mit einer Zinkanode und dem als Kathode angeschlossenen Metallsubstrat, gekennzeichnet durch die Stufen, dass man dieses Substrat in gereinigtem Zustand in einen mindestens 40 g/I Zinkionen und 30-110 g/I unlöslichen losen Graphit enthaltenden Säure/Zink-Galvanisierelektrolyten bei pH 5-5,7 eintaucht, diese Elektrolysezelle unter ständigem Aufrühren des Graphits zu einer durch den ganzen Elektrolyten gleichförmigen Suspension mit einer solchen Stromdichte beaufschlagt, dass sich Zink ohne Anbrennen auf jener Oberfläche abscheidet, und dieses Aufrühren von Zeit zu Zeit unterbricht, um diesen Graphit such absetzen und mit besagtem, sich auf jener Kathode abscheidenden Zink vermischen zu lassen, wobei der kombinierte Niederschlag aus Zink und Graphit auf diesem Substrat gleichförmig verteilten Graphit in einer Menge von 30-48 Gew.-% des kombinierten Niederschlags enthält und bei einer plattierten Dicke von 0,00127 cm (0,0005 Zoll) einen Reibungsbeiwert von 0,130 oder kleiner, nach mindestens 72 Stunden in einer Salzsprühnebelumgebung keinen roten Rost und nach vier Monaten in einer Schwefeldioxyd enthaltenden industriellen Umgebung keine Zerstörug durch Korrosion zeigt.

2. Verfahren nach Anspruch 1, wobei besagtes Aufrühren von Zeit zu Zeit 15 bis 60 Sekunden Lang in Abständen von 15 bis 180 Sekunden unterbrochen wird.

3. Verfahren nach Anspruch 1 oder 2, worin dieser lose Graphit eine durchschnittliche Teilchengrösse von 1 bis 25 Mikron aufweist.

4. Verfahren nach einem der Ansprüche 1 bis 3, worin als Elektrolyt ein saurer Chloridtyp vorliegt, der entweder durch Zusatz von 70-85 g/I Zinkchlorid zu 100-150 g/I Kaliumchlorid oder 45-110. g/I Zinkchlorid zu 100-200 g/I Natriumchlorid bereitet wird und ferner 26―40 g/I Borsäure enthält.

5. Verfahren nach Anspruch 4, worin dieser Elektrolyt zusätzlich 0,4-1 g/1 Gelatine enthält.

6. Verfahren nach Anspruch 4, worin dieser Elektrolyt zusätzlich 0,1-4,0 g/I Kokosaminacetat enthält.

7. Verfahren nach einem der vorhergehenden Ansprüche, worin diese Elektrolysezelle mit einer Stromdichte von 0,1-2,0 A/dm² (1-20 A pro Quadratfuss) beaufschlagt wird.

8. Verfahren nach einem der vorhergehenden Ansprüche, worin jenes Aufrühren durch pulsierte Einführung von Luft in diesen Elektrolyten erfolgt.

9. Verfahren nach einem der vorhergehenden Ansprüche, worin man diesen Elektrolyten bei einer Temperatur von 24-32°C (75-90°F) hält.

10. Verfahren nach einem der vorhergehenden Ansprüche, worin dieses Metallsubstrat aus der Stahl, Kupfer, Nickel, Messing, Bronze, Zink und Aluminium sowie Leitfähige Kunststoffe umfassenden Gruppe ausgewählt ist.

11. Verfahren nach einem der vorhergehenden Ansprüche, wobei man zusätzlich jenes zusammen abgeschiedene Material für einen Zeitraum von 10-30 Sekunden in eine Chromatlösung eintaucht, um darauf einen aus Zinkchromat bestehenden Umwandlungsüberzug zu bilden.

12. Verfahren nach einem der vorhergehenden Ansprüche, worin als solches Substrat ein Metallverschluss mit Gewinde vorliegt.

13. Verfahren nach Anspruch 12 zum Galvanisieren einer Charge von Metallverschlüssen mit Gewinde unter Verwendung eines Fassgalvanisierapparats mit einem durchlochten Fass, in den der Galvanisierelektrolyt mit den als Kathode .angeschlossenen Verschlüssen eingeführt wird, dadurch gekennzeichnet, dass man diese in dem Fass befindlichen Verschlüsse nacheinander in eine Reihe von Behältern eintaucht, die eine alkalische Reinigungslösung, eine Wasserspülung, eine Beizlösung zur Entfernung von Oxyden, eine Wasserspülung, den Zink/Graphitgalvanisierelektrolyten bzw. eine Wasserspülung enthalten, diesen Zink/Graphitgalvanisierelektrolyten mit Strom beaufschlagt, wenn diese im Fass befindlichen Verschlüsse in jene Lösung eingetaucht sind, wobei eine solche Strommenge zugeführt wird, dass sich Zink auf diesen Verschlüssen ohne Anbrennen abscheidet, wobei während der Abscheidung Druckluftstrahlen eingeführt werden, um den Graphit ständig in diesem Elektrolyten in Suspension zu halten, und wobei besagte Drehung des Fasses und das Aufrühren mit Luft von Zeit zu Zeit unterbrochen werden, um den Graphit wandern und sich mit besagtem Zink auf der Kathode abscheiden zu lassen.

## Revendications

1. Procédé de dépôt électrolytique de zinc et de graphite sur un support métallique conducteur, par l'utilisation d'une cellule électrolytique comportant une anode de zinc et le support métallique connecté en tant que cathode, procédé comprenant les étapes d'immersion dudit support, nettoyé, dans un électrolyte de zingage acide, contenant au moins 40 g/litre d'ions zinc et 30-110 g/litre de graphite insoluble en vrac, ledit électrolyte ayant un pH de 5-5,7, et d'alimentation de ladite cellule électrolytique avec une densité de courant suffisante pour qu'il y ait dépôt de zinc sur ladite surface sans brûlage, tout en agitant en continu ledit graphite en une suspension homogène dans l'ensemble dudit électrolyte, ladite agitation étant périodiquement interrompue pour permettre audit graphite de se déposer et se mélanger avec ledit zinc à mesure que celui-ci se dépose à ladite cathode, la couche de zinc et de graphite déposés simultanément sur ledit support contenant du graphite réparti de façon homogène en une quantité de 30-48% en poids, par rapport à la couche formée par dépôt simultané, ayant un coefficient de frottement égal ou inférieur à 0,130, pour une épaisseur de dépôt de 0,00127 cm ne montrant pas de formation de rouille dans en environnement de brouillard salin pendant.au moins 72 heures, et pas de destruction due à la corrosion après 4 mois dans un environnement industriel contenant de l'anhydride sulfureux.

2. Procédé selon la revendication 1, dans lequel ladite agitation est périodiquement interrompue pendant des périodes de 15 à 60 secondes, à intervalles de 15 à 180 secondes.

3. Procédé selon la revendication 1 ou 2, dans lequel ledit graphique en vrac a une taille moyenne de particules de 1 à 25 µm.

4. Procédé selon l'une quelconque des revendications 1 à 3, dans lequel ledit électrolyte est du type chlorure acide obtenu par addition de soit 70-85 g/litre de chlorure de zinc avec 100-150 g/litre de chlorure de potassium, soit de 45-110 g/litre de chlorure de zinc avec 100-200 g/litre de chlorure de sodium, ledit électrolyte contenant également 26―40 g/litre d'acide borique.

5. Procédé selon la revendication 4, dans lequel ledit électrolyte contient en outre 0,4-1 g/litre de gélatine.

6. Procédé selon la revendication 4, dans lequel ledit électrolyte contient en outre 0,1-4,0 g/litre d'acétate de cocamine.

7. Procédé selon l'une quelconque des revendications précédentes, dans lequel ladite cellule électrolytique est alimentée par une densité de courant de 0,1-2,0 A/dm².

8. Procédé selon l'une quelconque des revendications précédentes, dans lequel ladite agitation est réalisée par utilisation d'air pulsé dans ledit électrolyte.

9. Procédé selon l'une quelconque des revendications précédentes, dans lequel ledit électrolyte est maintenu à une température de 24―32°C.

10. Procédé selon l'une quelconque des revendications précédentes, dans lequel ledit support métallique est choisi parmi l'acier, le cuivre, le nickel, le laiton, le bronze, le zinc et l'aluminium, ainsi que des matières plastiques conductrices.

11. Procédé selon l'une quelconque des revendications précédentes, dans lequel ledit procédé comprend en outre l'étape d'immersion du matériau Co-dépose dans une solution de chromate pendant une durée de 10-30 secondes, pour former une couche de conversion constituée de chromate de zinc sur la couche formée par dépôt simultané.

12. Procédé selon l'une quelconque des revendications précédentes, dans lequel ledit support est un élément métallique de fixation fileté.

13. Procédé selon la revendication 12 de revêtement électrolytique d'un lot d'éléments métalliques de fixation filetés, par l'utilisation d'un appareil de dépôt électrolytique en tonneau, comportant un tonneau perforé dans lequel est introduit l'électrolyte de dépôt électrolytique ainsi que les éléments de fixation connectés de manière à constituer une cathode, procédé comprenant l'immersion dudit tonneau contenant les éléments de fixation, successivement dans une série de cuves, les cuves comprenant une solution caustique de nettoyage, de l'eau de rinçage, une solution de décapage pour l'élimination d'oxydes, de l'eau de rinçage, l'électrolyte pour le dépôt de zinc et de graphite, et de l'eau de rinçage; l'alimentation dudit électrolyte pour le dépôt de zinc et de graphite lorsque lesdits éléments de fixation contenus dans le tonneau sont plongés dans ladite solution, ladite alimentation étant effectuée à un niveau permettant le dépôt de zinc sur lesdits éléments de fixation sans brûlage, ledit dépôt étant effectué avec l'injection de jets d'air comprimé pour maintenir le graphite constamment en suspension dans ledit électrolyte; et l'interruption périodique de ladite rotation du tonneau et de l'agitation au moyen de l'air, pour permettre audit graphite de migrer et de se déposer avec ledit zinc sur la cathode.
